

1

3,756,773

COLORING SYNTHETIC HYDROPHOBIC FIBERS  
WITH ARALKYL SUBSTITUTED PHENOLS  
Jayanti Isharani, Dobbs Ferry, N.Y., assignor to  
Ciba-Geigy Corporation, Greenburgh, N.Y.  
No Drawing. Filed Aug. 2, 1971, Ser. No. 168,385  
Int. Cl. D06p 5/04

U.S. CL. 8—173

1 Claim

### ABSTRACT OF THE DISCLOSURE

A technique is disclosed for coloring hydrophobic textile fibers, particularly polyester fibers with a disperse dyestuff employing ortho-benzyl para-chloro phenol.

### BACKGROUND OF THE INVENTION

The present invention is directed to a process of dyeing and printing hydrophobic organic polymers with disperse or basic dyestuffs utilizing a carrier component of an aralkyl substituted phenol, substituted halophenol, or the salts thereof.

It is well known in the prior art techniques of dyeing and printing that special procedures are necessary to color a textile structure or fabric that is water impermeable since otherwise serious problems arise. For example, with many conventional techniques, the dyestuff does not penetrate the water impermeable material and does not affect coloration should coloration occur, it is not of a permanent nature and leaches out during a subsequent washing step.

To circumvent the problems of the noncoloration or the leaching of the dye, the prior art has employed in the treatment of the hydrophobic synthetic fibers elevated pressures with temperatures greater generally than 250° F. Generally speaking, dyeing under pressure at elevated temperature is undesirable due to the expense and complex procedures employed. To bypass this dyeing technique, the prior art has also turned to specific carrier components. These carriers aid in the penetration of the dye into the fiber by causing a swelling of the base substrate.

The use of carriers in dyeing techniques upon hydrophobic fibers allows satisfactory results as temperatures as low as 200 to 210° F. although a temperature of 212° F. at normal atmospheric pressure is preferred. There are many carrier components for hydrophobic fibers known in the prior art to be employed with a variety of dyes. Nevertheless many of these carrier components have some drawbacks such as lack of availability, undue toxicity, lack of ease of removal from the substrate, effect on lightfastness of color, or influence of buildup of a heavy shade.

It is an object of this invention to provide a novel carrier component which is suitable for dyeing hydrophobic material.

### DESCRIPTION OF THE INVENTION

In accordance with the present technique of this invention dyeing and printing of synthetic hydrophobic fiber utilizes a disperse or basic dyestuff in conjunction with an emulsion of a carrier component of an aralkyl substituted phenol, substituted halophenol as well as its water soluble salts. This carrier is of the following formula:



wherein R<sub>1</sub> represents an aralkyl group and R<sub>2</sub> represents hydrogen or a halogen. Illustratively, the salts of the aralkyl substituted phenol or substituted halophenol are

2

formed when the carrier component is in the aqueous dyebath environment. In the above formula an example of a desirable aralkyl is benzyl while an example of a desirable halogen is chlorine.

5 The types of dyestuffs employable in the present invention are well known in the art as disperse and basic dyestuffs. Illustratively although not limiting of suitable disperse dyestuffs are those listed in the Color Index under the Disperse dye classification. Basic dyes that may 10 be used include those listed in the Color Index under the basic dye classification.

There are various techniques and procedures for dyeing the synthetic fibrous material utilizing the disperse or basic dyestuff and carrier component disclosed herein. 15 As employed herein, a fibrous material includes fibers, yarns, threads, fabric ribbons, tapes and tabs. The disperse dyestuff and emulsified carrier may be added to a bath at temperature equivalent to the boiling point of water. A time interval of two or three hours is utilized during 20 which time the fibrous substrate is contacted with the dyebath composition. Thereafter the fabric is washed followed by drying.

Another technique of applying the dispersed dyestuff in emulsified carrier is with a composition containing the dyestuff carrier and emulsifying agent which is applied by padder on the substrate followed by steaming for a time period of ten or fifteen minutes.

Insofar as printing techniques are concerned printing may be carried out in the usual way by adding the carrier emulsion to a paste and printing the material on a roller or screen printing unit followed by fixing the dye by exposing to steam or heat treatment.

A thermosol technique may be utilized by padding the material with a mixture of a disperse dye-emulsified carrier of the type disclosed herein followed by drying at 35 100 to 250° C. for 1 to 30 minutes. Alternatively thermofixing may take place with steam injection at temperature-time conditions as 340° F. for 1 to 30 minutes.

The types of substrates that may be employed as previously disclosed are hydrophobic materials that do not color readily without the use of a carrier component. Suitable examples of the hydrophobic material include polyester and acid modified polyester, polyamide, cationic dyeable polyamide, polypropylene, polyacrylonitrile, and its modified versions, modacrylics, or triacetate.

The amount of carrier component of the type disclosed herein may vary within wide limits and depends primarily on the dry weight of the hydrophobic material being dyed. The limit of the carrier components are broad and may 50 be from 0.1 to 30% by weight of the active carrier contents. A more preferred range will be between 1 to 10% by weight.

The above mentioned carrier of this invention is not restricted to being applied alone but can be incorporated 55 with other carriers such as o-phenol phenyl, biphenyl, chlorinated hydrocarbons, salicylates, alkyl benzoates, methyl naphthylene such as to an extent of 50% by weight of the disclosed carrier and thus conserve the original characteristics of the aralkyl substituted phenols or halo-phenols or their water soluble salts respectively.

It is also within the scope of the present invention that a solvent of the carrier component be employed. For example, glycols and glycol ethers are suitable for the carrier component. Illustratively for ortho-benzyl para-chloro phenol suitable solvents include 2-phenoxy ethanol and p-chloro-2-phenoxy ethanol.

65 To further illustrate the innovative aspects of the present invention the following examples are provided:

#### Example 1

The dye carrier is prepared by mixing 80 parts  $\beta$ -ortho-benzyl-para-chloro phenol and 20 parts sulfated nonyl

poly (ethylene oxy) ethanol, 30 g./l. of this emulsion is mixed with 10 g./l. of a gum (Polygum 260) and 10 g./l. of dyestuff of the following formula



A polyester carpet is padded with this mixture on Kuster padder (wet pickup 300%) and is steamed in Kuster steamer for 12 minutes. A yellow shade is obtained with good general fastness.

Example 2

A dye carrier is prepared from 70 parts ortho benzyl para-chloro phenol, 10 parts methyl salicylate and 20 parts dioctyl sulfosuccinate. 30 g./l. of this emulsion is mixed with 10 g./l. polygum 260 and 10 g./l. dyestuff of the following formula:



The procedure of dyeing is the same as in Example 1.

Example 3

The technique of Example 2 is followed but with the following dyestuffs mixture and a steaming time of 10 minutes:

|                                         | G./l. |
|-----------------------------------------|-------|
| C.I. Disperse Red 80                    | 8     |
| C.I. Disperse Orange 37 (a monoazo dye) | 8     |
| C.I. Disperse Red 65 (a monoazo dye)    | 0.7   |

A dark red is obtained with very good lightfastness.

Example 4

A printing paste is utilized which contains a 4% carrier emulsion of Example 1 with 3% alginate thickener and 1% of the dyestuff formula:



After printing, the substrate is submitted to a 30 minute steaming at 20 lb. pressure. After rinsing and soaping a strong blue is obtained, with good fastness properties.

Example 5

The procedure is the same as Example 4 but is printed on polyester carpet and heat set 1½ minutes at 350° F.

Example 6

The procedure of Example 5 is followed except in the carrier emulsion, a carrier mixture of 90 parts of o-benzyl para-chloro phenol and 10 parts p-chloro-2-phenoxy ethanol is used.

Example 7

15 A carpet of acid modified polyester, trade name "Fortrel 404" is dyed according to Example 2 with 5 g./l. of dyestuff of the following formula:



A good red is obtained with good lightfastness.

Although the present invention has been shown and described with reference to particular embodiments, it is understood the invention is designed only by the scope of the attached claim.

What is claimed is:

1. In a process for coloring polyester fibrous material with a disperse dyestuff with the aid of a carrier component, the improvement comprising utilizing as a carrier component ortho-benzyl para-chloro phenol.

References Cited

UNITED STATES PATENTS

2,743,991 5/1956 Schoonover ----- 8—173 X  
3,702,229 11/1972 Campana ----- 8—173

FOREIGN PATENTS

1,000,407 11/1972 Great Britain.  
1,142,338 4/1963 Germany ----- 8—175

OTHER REFERENCES

J. Valentine, J. Polymer Sci., vol. XXIII, pp. 297-314.

DONALD LEVY, Primary Examiner

U.S. Cl. X.R.

50 8—169, 168, 175, 21 C